

## UNITED STATES PATENT OFFICE

2,054,894

## IMBEDDING MASS FOR DENTAL PURPOSES

Werner Busch, Dormagen, and Paul Wolski,  
Leverkusen-Wiesdorf, Germany, assignors to  
Winthrop Chemical Company, Inc., New York,  
N. Y., a corporation of New York

No Drawing. Application November 27, 1933,  
Serial No. 700,020. In Germany December 1,  
1932

5 Claims. (CL 22—188)

This invention relates to an imbedding mass for dental purposes which is characterized by yielding dental molds of high power of thermal expansion and of sufficiently great hardness, particularly in the heated state of the mold.

The known imbedding masses for dental purposes merely consist of a mixture of plaster of Paris and quartz-like materials, such as sand, silica, kaolin and the like. Apart from a great 10 fineness of the mass which is necessary to obtain a smooth surface of the mold a power of thermal expansion as high as possible, and a sufficiently great hardness, particularly when the mold is heated to the casting temperature, are required especially when the molds are intended for the 15 manufacture of gold casts. The high power of thermal expansion is necessary to compensate the contraction of the gold after the cast has been made; the great hardness of the mold is required to avoid brittling and the deformation 20 of the mold when the heavy liquid gold flows in.

The imbedding masses hitherto known and marketed yield molds which possess the high power of thermal expansion and a great hardness 25 simultaneously only to an unsatisfactory extent. The power of thermal expansion may be increased in a known manner by adding a greater percentage of the quartz-like material to the imbedding mass, however, the solidity and stability of the mold is strongly diminished by such a procedure. On the other hand, an increase of the contents 30 of plaster of Paris by which a greater solidity is attained unfavorably influences the power of thermal expansion. For the said reasons it has 35 hitherto been impossible to prepare molds for dental purposes which yield unobjectionable and undamaged casts which do not show the effect of the contraction of the casting material. Wearisome experiments have been made to compensate the contraction of casting material by 40 utilizing a certain expansion of the wax model while imbedding the wax model at elevated temperature. Such procedure, however, is practically very unsatisfactory.

45 The present invention provides for an imbedding mass which yields molds displaying simultaneously high power of thermal expansion and great hardness, so that the contraction of the casting material is compensated during the manufacture of the cast, and undamaged casts are obtained.

In accordance with the present invention an imbedding mass yielding the said dental molds of high power of thermal expansion and great hardness is obtainable by evenly distributing in the

hitherto customary imbedding masses, mainly consisting of plaster of Paris and a quartz-like material, a relatively small percentage of a solid organic acid, such as citric acid, tartaric acid, oxalic acid, succinic acid, gluconic acid, benzoic acid, salicylic acid and naphthoic acid. Relatively small quantities of the organic acids are required to bring about the above described effects. Preferably the said substances are added in a percentage of about 1% or less, but it may 10 be mentioned that also 5% may be added without any remarkable disadvantage. The said organic acids may be used in admixture with each other. The addition of the said organic acids causes the great hardness and favorably 15 influences the expansion of the mass.

The new imbedding mass characterized by the contents of the solid organic acids may contain other additions usual in the manufacture of imbedding masses, for instance, substances which 20 accelerate the solidification of the mold, such as potassium chloride and potassium sulfate, sodium chloride and sodium sulfate, potassium-aluminum sulfate; or retarding additions, for instance, borax, in order to regulate the setting 25 time of the imbedding mass as desired. Other customary additions are, for instance, coloring substances, in order to better differentiate the imbedding mass from other substances.

It may be mentioned that an imbedding mass 30 yielding molds of particularly favorable properties as to solidity and expansion are obtainable when using instead of the alabaster plaster of Paris, customary in such imbedding masses, wholly or partially a semi-hydrate gypsum which 35 is obtainable by heating natural gypsum in a closed vessel at an elevated pressure, and which is characterized by a particularly high shaking weight, for instance, a shaking weight "loosely put in" of above 0.9 "g./ccm." and "shaken in" of 40 above 1.45 "g./ccm." and a strewed in quantity" of more than 230 grams of the plaster of Paris, the said "strewed in quantity" being defined as that quantity of a gypsum which, when strewed into 100 ccs. of water, still yields a mass which 45 is capable of being poured. The method of determining the "shaking weight" (sometimes also called "weight by volume") "loosely put in" and "shaken in" is the usual one. The gypsum is poured into a funnel with a sieve placed therein, 50 and runs into a vessel of a content of 1 liter. The height and the diameter of the vessel are in a proportion of 2:3. The gypsum beyond the rim of the container is removed by striking. During this operation any shaking of the container is to 55

be avoided. The content of the container is then weighed. The weight in kg. per liter determines the shaking weight "loosely put in". If the content of the container is shaken during the running of the gypsum from the funnel until the container is completely filled so that no more gypsum may be added and the gypsum beyond the rim of the container is again removed by striking, the container then gives the shaking weight "shaken in".

10 The molds obtainable by means of the above described imbedding masses permit in a very simple manner the manufacture of dental casts, for instance, gold casts, which practically do not 15 show any deviation from the model since the molds prepared from the new imbedding mass compensate the normal contraction of the cast material in view of their high thermal expansion during the casting process. It is obvious that 20 this simple means for avoiding the breaking of the mold and the contraction of the cast constitutes a remarkable advance in the manufacture of dental casts.

25 The invention is further illustrated by the following example, but it is not restricted thereto:—

30 *Example.*—30 parts by weight of a semi-hydrate gypsum of good quality are well mixed with 65 parts by weight of finely ground quartz sand, 0.2 parts by weight of citric acid, 0.2 parts by weight of oxalic acid, and 0.1 part by weight of potassium sulfate. An imbedding mass is thus obtained 35 which yields in a favorable setting time (about 15–20 minutes) molds of great solidity in the heated state and of a high power of thermal expansion which practically compensates the contraction of gold (amounting to about 1.3% in a linear direction) when cooled from the melting temperature to normal temperature.

40 In the above case the semi-hydrate-gypsum is preferably wholly or partially a gypsum having a shaking weight "loosely put in" of above 0.9 and "shaken in" of above 1.45 and a "strewed in quantity" of about 230 grams. For instance, 45 the use of a mixture of 10 parts by weight of the normal alabaster plaster of Paris and about 25

parts by weight of the semi-hydrate gypsum having the properties above specified has proved to be very favorable.

5 The addition of potassium sulfate used as an accelerator for the solidification of the mold may be omitted, but also larger quantities of, for instance, 0.2 grams or of other accelerators mentioned above may be employed.

We claim:—

1. An expansive imbedding mass for dental purposes, comprising plaster of Paris and a finely divided quartz-like material, which imbedding mass is characterized by the content of a slight percentage of a solid organic carboxylic acid sufficient to give the mass an acid reaction when 15 mixed with water.

2. An expansive imbedding mass for dental purposes, comprising plaster of Paris and a finely divided quartz-like material, which imbedding mass is characterized by the content of a slight 20 percentage of a solid organic polycarboxylic acid sufficient to give the mass an acid reaction when mixed with water.

3. An expansive imbedding mass for dental 25 purposes, comprising plaster of Paris and a finely divided quartz-like material, which imbedding mass is characterized by the content of a slight percentage of oxalic acid sufficient to give the mass an acid reaction when mixed with water.

4. An expansive imbedding mass for dental 30 purposes, comprising plaster of Paris and a finely divided quartz-like material, which imbedding mass is characterized by the content of a slight percentage of oxalic and citric acid sufficient to 35 give the mass an acid reaction when mixed with water.

5. An expansive imbedding mass for dental 40 purposes, comprising about 60 parts by weight of fine quartz sand, about 30 parts by weight of a semi-hydrate-gypsum, about 0.2 parts by weight of citric acid and 0.2 parts by weight of oxalic acid, said imbedding mass giving an acid reaction when mixed with water.

WERNER BUSCH.  
PAUL WOLSKI.